

# United States Patent

[19]

Grannen

[11] 3,768,646

[45] Oct. 30, 1973

[54] FLOTATION OF SILICEOUS MATERIALS  
WITH DIAMINE REACTION PRODUCTS

[75] Inventor: Edward A. Grannen, Upland,  
Calif.

[73] Assignee: Occidental Petroleum Corp.,  
Los Angeles, Calif.

[22] Filed: Sept. 16, 1971

[21] Appl. No.: 181,233

## Related U.S. Application Data

[62] Division of Ser. No. 467, Jan. 2, 1970, abandoned.

[52] U.S. Cl. .... 209/166, 260/404.5

[51] Int. Cl. .... B03d 1/02

[58] Field of Search..... 209/166; 260/404.5

[56]

## References Cited

### UNITED STATES PATENTS

2,267,205 12/1941 Kyrides..... 209/166

|           |        |                    |           |
|-----------|--------|--------------------|-----------|
| 2,329,149 | 9/1943 | Weiner .....       | 209/166   |
| 2,494,132 | 1/1950 | Jayne .....        | 209/166   |
| 2,569,417 | 9/1951 | Jayne .....        | 209/166   |
| 2,805,135 | 9/1957 | Bell.....          | 260/404.5 |
| 2,927,692 | 3/1960 | Hollingsworth..... | 209/167   |

Primary Examiner—Robert Halper  
Attorney—Christie, Parker & Hale

[57]

## ABSTRACT

A process for the flotation separation of ore values from siliceous materials by reagents obtained by the reaction of N,N-dialkyl alkylene diamines and N,N-dialkyl-N'-alkyl alkylene diamines with saturated, unsaturated and hydroxylated fatty acids.

3 Claims, No Drawings

## FLOTATION OF SILICEOUS MATERIALS WITH DIAMINE REACTION PRODUCTS

mixture thereof, at a temperature of from about 130° C to about 260° C for a time sufficient for the condensation reaction to occur.

The amine reaction product formed and their salts are unusually selective reagents for the beneficiating separation of ore values, such as phosphate rock, from siliceous materials.

### DESCRIPTION

According to the present invention, there is provided a new class of fatty acid amines which are highly selective beneficiation reagents for the removal of siliceous materials from mineral ores.

The amine reagents of this invention are prepared, in general, by reaction of saturated, unsaturated and hydroxylated fatty acids or mixtures thereof with at least one monofunctional diamine having the general formula:



wherein R is hydrogen or an alkyl group and R/R'' and R''' are independently alkyl groups. The alkyl groups present may be straight chained or branched and preferably contain from about 1 to about 4 carbon atoms.

Illustrative but no wise limiting of the monofunctional N,N-dialkyl alkylene diamines and N,N-dialkyl-N'-alkylenediamines which may be used in accordance with the practice of this invention there may be mentioned N,N-diethylethylene diamine; N,N-diethyl-N'-methylethylene diamine; N,N-dimethyl-1,2-propane diamine; N,N-diethyl-1,3-propane diamine; N,N-dimethyl-1,3-propane-diamine; N,N-dimethylethylene diamine and the like.

In addition to at least one monofunctional N,N-dialkyl alkylene diamine or N,N-dialkyl-N'-alkyl alkylene diamine, there may be present in the reaction system, reactive polyfunctional amines such as alkylene diamines, polyalkylene diamines, polyalkylene polyamines and the like. The amounts which may be present, generally, range from about 0.6 to about 1.5 mol per mol of monofunctional diamine.

The saturated, unsaturated or hydroxylated fatty acids which may be reacted with an amine system containing N,N-dialkyl alkylene diamines and N,N-dialkyl-N'-alkyl alkylene diamines to provide the novel reagents of this invention may be varied widely. Preferably, however, they contain on the average, from about 8 to about 26 carbon atoms in the chain and may be derived from the fats or oils of either vegetable or animal origin.

Illustrative, but no wise limiting of the basic acid constituents which may be present in the fatty acids employed in accordance with the practice of this invention, there may be mentioned caprylic, pelargonic, capric, undecanoic, lauric, tridecanoic, myristic, pentadecanoic, palmitic, margaric, stearic, nonadecanoic, arachidic, heneicosanoic, behenic, tricosanoic, lignoceric, pentacosanoic, cerotic, oleic, linoleic and the like.

As indicated, the acids may be synthetic or derived from natural vegetable or animal origins. Specific ex-

amples but no wise limiting of naturally occurring acids, which are usually mixtures of one or more of the above acids, there may be mentioned coconut oil acid, palm oil acid, cottonseed oil acid, corn oil acid, fish oil acid, peanut oil acid, soy bean oil acid, linseed oil acid, tall oil acid and the like.

As indicated, the amount of acid employed for the condensation reaction is an amount sufficient to provide from about 0.9 to about 3.7, preferably from about 10.0 to about 2.0 molar equivalent saturated, unsaturated fatty or hydroxylated fatty acid for each primary or secondary amine available in the reaction system.

Accordingly, each of the N,N-dialkyl alkyl diamines and N,N-dialkyl-N'-alkyl alkylene diamines provided in 15 the reaction system in accordance with the practice of this invention provide one functional group for reaction with each molar equivalent of the fatty acid. Where polyfunctional amines, such as those set forth above, are present, a fatty acid equivalent, within the 20 range prescribed above, should be provided for each amine group in the system having an active hydrogen, namely the primary and secondary amines.

Novel reagents provided in accordance with the practice of this invention are typically obtained by condensing the mixture of the fatty acid amines at a temperature from about 130° to about 260° C for a period of time sufficient for the system to complete the reaction. Generally, depending on the mixture, condensation time from about 2 to about 6 hours or more will be required.

The properties of the condensation product obtained will vary somewhat depending upon the provided mol ratio of acid to amine. At lower mol ratios a condensation product will readily dissolve in water. At higher acid ratios, however, the product behaves generally more like the fatty acid used and shows a tendency to disperse rather than dissolve in solution.

The tertiary amine groups are present in the amine condensation products of this invention and have been 40 observed to provide the amine reaction products with selective activity for separating of ore values, such as phosphate rock, from siliceous materials by froth flotation.

The tertiary amine groups also provide a functionality which allows the formation of salts by reaction with acids such as formic acid, acetic acid, propionic and hydrochloric acid, hydrofluoric acid and the like, to provide salts in which the novel fatty acid amines of this 45 invention serve as a cation and where the anion is provided by the acid. These salts are also active reagents for the beneficiation of ores and are particularly selective reagents for the flotation separation of ore values from siliceous materials.

Although they may be used alone in the beneficiation 55 of mineral values, the activity of the amine reagents of this invention may be further promoted by the presence of certain acid like petroleum derivatives such as kerosene and the like in the system where flotation is carried out. They may also be used in conjunction with other beneficiating reagents for the separation of values from ores and the like.

The amount of the amines of this invention employed in the beneficiation of ores is not narrowly critical. Generally, amounts from about 0.1 to about 2.0 or more pounds per ton of ore beneficiated may be used.

While no wise limiting, the following are examples of the preparation of the novel fatty acid amines of this

invention as well as their use as flotation reagents for the beneficiation of orcs.

#### EXAMPLES 1 TO 15

A series of fatty acid-amine condensation reactions carried out using a reactor equipped with a stirrer, a condenser and a temperature indicator. In each instance, the amine and acid were added in specified amounts to the reactor and the mixture heated with agitation. An initial temperature increase was generally observed when the amine and the fatty acid were mixed. With additional heating, water began to distill off at a temperature from between 140° and 150° C and continued to evolve until the temperature of the reaction mass reached about 220° to 230° C. Reaction times varied from about 3 to about 6 hours. The nature of the amine fatty acids systems reacted and the mol ratios employed and general properties of the reaction mass obtained are shown in Table I.

10

The amine reagent prepared in Example 9 was used in place of amine prepared in Example 2. Florida phosphate rock was treated using amine in the concentration of 0.45 lb. per ton of phosphate rock with kerosene as a frother. Results of this beneficiation separation are shown in Table IV:

TABLE IV

| Concen-<br>trate | Wt.%  | Assay | BPL   | Insol.<br>Assay |   |
|------------------|-------|-------|-------|-----------------|---|
|                  |       |       |       | Distr.          | — |
| Tails            | 84.7  | 73.9  | 97.6  | 3.7             |   |
| Heads            | 15.3  | 10.0  | 2.4   | —               |   |
|                  | 100.0 | 64.1  | 100.0 |                 |   |

## 15

## EXAMPLE 19

The amine prepared in Example 1 was used to treat a rougher phosphate rock containing about 10 percent

TABLE I

| Example | Fatty acid source               | Wt. percent | Amine                                                       | Wt. percent | Mole ratio acid amine | Remarks                                |
|---------|---------------------------------|-------------|-------------------------------------------------------------|-------------|-----------------------|----------------------------------------|
| 1       | Tall oil <sup>1</sup>           | 84          | N,N-dimethyl-1,3-propane diamine                            | 16          | 1.82                  | Opaque solution—two layers in standing |
| 2       | do                              | 78          | do                                                          | 22          | 1.20                  | Clear brown solution.                  |
| 3       | do                              | 91.5        | do                                                          | 8.5         | 3.68                  |                                        |
| 4       | do                              | 88          | do                                                          | 12          | 2.50                  | Soluble at 40%.                        |
| 5       | do                              | 86.6        | do                                                          | 13.4        | 2.28                  | Solids separation on standing.         |
| 6       | do                              | 82.8        | do                                                          | 17.2        | 1.54                  | Opaque solution—no phase separation.   |
| 7       | Oleic acid                      | 84          | do                                                          | 16          | 1.9                   | Clear, light yellow solution.          |
| 8       | Tall oil heads <sup>2</sup>     | 84          | do                                                          | 16          | 1.83                  | Opaque solution.                       |
| 9       | do                              | 77.8        | do                                                          | 12.2        | 1.21                  | Insoluble.                             |
| 10      | do                              | 91.4        | do                                                          | 8.6         | 3.64                  | Opaque brown solution.                 |
| 11      | Distilled tall oil <sup>3</sup> | 84          | do                                                          | 16          | 1.83                  |                                        |
| 12      | Tall oil                        | 77.7        | { N,N-dimethyl-1,3-propane diamine<br>{ Diethylene triamine | 11.1        | 1.21                  |                                        |
| 13      | do                              | 84.5        | { N,N-dimethyl-1,3-propane diamine<br>{ Diethylene triamine | 6.2         |                       |                                        |
| 14      | do                              | 84.7        | { N,N-dimethyl-1,3-propane diamine<br>{ Diethylene triamine | 9.3         | 1.92                  |                                        |
| 15      | Tall oil heads                  | 84.5        | { N,N-dimethyl-1,3-propane diamine<br>{ Diethylene triamine | 9.7         | 1.92                  |                                        |
|         |                                 |             |                                                             | 6.2         |                       |                                        |
|         |                                 |             |                                                             | 9.3         |                       |                                        |

<sup>1</sup> Union Camp Corporation CX-1, reconstituted tall oil.

<sup>2</sup> Arizona Chemical Company, Acintol H-2122.

<sup>3</sup> Arizona Chemical Company, Acintol D-29LR.

## EXAMPLE 16

The amine reagent prepared in Example 2 was used as a beneficiation reagent for the cleaner float of a Florida phosphate rock containing 10 percent insolubles in a concentration of 0.3 lb. per ton of phosphate rock. Kerosene was present as a frother. The results of the froth flotation separation are shown in Table II:

TABLE II

| Concen-<br>trate | Wt.%  | Bone Phosphate of Lime<br>Assay (% P <sub>2</sub> O <sub>5</sub> ) | Distr. (%) | Insol.<br>Assay, % |   |
|------------------|-------|--------------------------------------------------------------------|------------|--------------------|---|
|                  |       |                                                                    |            | Assay, %           | — |
| Concen-<br>trate | 84.5  | 72.8                                                               | 97.6       | 4.3                |   |
| Tails            | 15.5  | 9.7                                                                | 2.4        | —                  |   |
| Head<br>(Total)  | 100.0 | 63.0                                                               | 100.0      |                    |   |

## EXAMPLE 17

The procedure of Example 16 was repeated except the amine was used at a concentration of 0.45 lb. per ton of ore process. The results are shown in Table III:

TABLE III

| Concen-<br>trate | Wt. % | Assay (% P <sub>2</sub> O <sub>5</sub> ) | BPL  | Insol.<br>Assay, % |    |
|------------------|-------|------------------------------------------|------|--------------------|----|
|                  |       |                                          |      | Distr. (%)         | 65 |
| Concen-<br>trate | 84.1  | 73.7                                     | 97.3 | 4.0                |    |
| Tails            | 15.9  | 9.0                                      | 2.3  | —                  |    |
| Heads            | 100.0 | 63.1                                     | 99.6 |                    |    |

insolubles in a concentration of 0.5 lb. per ton. The results are shown in Table V:

TABLE V

| Concentrate | BPL, Wt.% | Insol. Wt.% | Yield, BPL |
|-------------|-----------|-------------|------------|
| Concentrate | 69.2      | 2.6         | 98%        |
| Tails       | 3.5       | 93.96       |            |

## EXAMPLE 20 - 21

The amine prepared in Example 2 was used for the beneficiation of phosphate at a high slurry density (22 - 23 percent) and compared to a commercial amine (Control A) which was a reaction product of a tall oil acid and diethylene triamine. As shown in Table VI, below, on a relative, comparative basis, phosphate loss in the tails was lower and insoluble retention by the float was also low.

TABLE VI

|                                           | Example 20 | Example 21 | Control A |
|-------------------------------------------|------------|------------|-----------|
| Amine, lbs./ton                           | 0.5        | 0.71       | 0.71      |
| Kerosene, lbs./ton                        | 0.96       | 0.96       | 0.96      |
| Fraction, P <sub>2</sub> O <sub>5</sub> % |            |            |           |
| Concentrate                               | 29.35      | 31.48      | 31.87     |
| Tails                                     | 2.83       | 1.98       | 2.43      |
| Acid. Insol. Wt. %                        |            |            |           |
| Concentrate                               | 5.64       | 8.03       | 8.44      |
| Tails                                     | 94.88      | 94.23      | 92.76     |

## EXAMPLE 22

The performance of the amine of Example 2 was

compared to the performance of an amine obtained by the condensation of tall oil acid with diethylene triamine at an acid to amine group ratio of approximately

1. The results are shown in Table VII wherein the amount of siliceous insolubles in the concentrate was reduced by 50 percent:

TABLE VII

|                                         | Example 22 | Control B |    |
|-----------------------------------------|------------|-----------|----|
| Amine, lbs./ton                         | 1.0        | 0.71      | 10 |
| Kerosene, lbs./ton                      | 1.2        | 1.2       |    |
| Fraction, P <sub>2</sub> O <sub>5</sub> |            |           |    |
| Concentrate                             | 32.65      | 31.58     |    |
| Tails                                   | 2.27       | 1.92      |    |
| Acid Insol., Wt. %                      |            |           |    |
| Concentrate                             | 3.54       | 6.70      |    |
| Tails                                   | 91.04      | 92.99     | 15 |

What is claimed is:

1. In a process for the flotation of siliceous materials from mineral values, the use as the flotation reagent for the siliceous materials, the condensation product obtained by reacting at least diamine having the structure:



wherein R is hydrogen or an alkyl group, R', R'' and R''' are independently alkyl groups and wherein each alkyl group contains from 1 to about 4 carbon atoms with from about 0.9 to about 3.7 mols per mol of primary and secondary amine groups of at least one fatty

acid selected from the group consisting of saturated, unsaturated and hydroxylated fatty acids containing from about 8 to about 26 carbon atoms.

2. A process as claimed in claim 1 in which the fatty acid in the reaction product is present in the amount of from about 1.0 to about 1.5 mols per mol of primary and secondary amine groups present in the reactive amine system.

3. In a process for the flotation of siliceous materials from mineral values, the use as the flotation reagent for the siliceous materials, the salt obtained by reacting the condensation product obtained by reacting at least diamine having the structure:



wherein R is hydrogen or an alkyl group R', R'' and R''' are independently alkyl groups and wherein each alkyl group contains from 1 to about 4 carbon atoms with from about 0.9 to about 3.7 mols per mol of primary and secondary amine groups of at least one fatty acid selected from the group consisting of saturated, unsaturated and hydroxylated fatty acids containing from about 8 to about 26 carbon atoms with an acid selected from the group consisting of formic acid, acetic acid, propionic acid, hydrochloric acid and hydrofluoric acid and wherein the anion of the salt is provided by the acid.

\* \* \* \* \*

35

40

45

50

55

60

65